

Aug. 5, 1930.

O. A. FREDERICKSON

1,772,436

ELECTRICAL CONDUCTOR

Filed Sept. 30, 1927



INVENTOR:

Otto A. Frederickson

BY *P. W. Hains.*

ATTORNEY

## UNITED STATES PATENT OFFICE

OTTO A. FREDERICKSON, OF WETHERSFIELD, CONNECTICUT, ASSIGNOR TO THE WIRE-MOLD COMPANY, OF HARTFORD, CONNECTICUT, A CORPORATION OF CONNECTICUT

## ELECTRICAL CONDUCTOR

Application filed September 30, 1927. Serial No. 223,005.

This invention relates to improvements in the construction of insulated electric conductors.

Insulated conductors as commonly constructed consist of a conductor wire having a rubber jacket over which is provided one or more layers of fibrous material, and it has been proposed heretofore to treat the fibrous layers with various compounds to render them moisture-proof and fire-repellant.

While the rubber jacket forms an excellent insulator for the conductor, it is not fire-repellant, and the rubber gradually deteriorates with the passage of time, becoming hard and inelastic. Furthermore, difficulty is sometimes experienced as a result of the fibrous covering slipping back off the rubber jacket to expose the latter.

Having in mind the foregoing the present invention relates to improvements in the construction of insulated conductors whereby the life of the rubber jacket is increased and the same is afforded better protection from fire and mechanical injury than heretofore. These desired results are obtained by applying a coating of stearin pitch or other fire-repellant compound directly to the outer surface of the rubber jacket, so that the pitch will form an air-tight coating over the rubber to prevent deterioration and hardening of the rubber due to oxidization and at the same time protect the rubber jacket from fire.

The various features of the invention will be best understood from the following description when read in connection with the drawings which illustrate one good practical form of the invention.

## In the drawings:

Fig. 1 is a perspective view of an electric conductor constructed in accordance with the present invention and having the several layers progressively removed;

Fig. 2 is a longitudinal sectional view of the conductor of Fig. 1; and

Fig. 3 is a transverse sectional view taken on the line 3-3 of Fig. 2.

The insulated electric conductor is shown in the drawings as having a conductor wire 10 about which is provided the usual rubber jacket 11, and in accordance with the pres-

ent invention the rubber jacket 11 is provided with a protecting coating 12 of stearin pitch or other sticky flame-retarding compound that will exclude air from the rubber jacket to reduce oxidization, and at the same time 55 protect this jacket from fire.

The coating compound 12 should have the properties of remaining resilient or flexible permanently so that it will not become hard and brittle upon the jacket as it ages, and it 60 preferably should be sufficiently sticky when applied to the rubber jacket to adhesively secure the covering 13, to be described, to the rubber jacket.

Stearin pitch forms an excellent protecting coating as it is fire-repellant to a high degree, due largely to its high melting point and its property of forming protecting blisters when exposed to fire, and it has the further property of remaining elastic or flexible 70 in all kinds of weather. Furthermore, it retains its plastic, rubbery character over a long period of time and is sufficiently adhesive to firmly adhere to the rubber jacket 11 and to the inner face of the protecting covering 13 to adhesively secure the covering 13 to the jacket 11.

The covering 13 is formed of fibrous material and may be braided, woven, or otherwise constructed, and is shown as a braid constructed of relatively large strands 14 of twisted paper which are interbraided with and secured in place by small strong strands 15.

It is desirable to render the protecting covering 13 water-proof so that the life of the covering and its insulating properties will not be reduced by the presence of moisture, it is also desirable to render the fibrous covering 13 fire-repellant to reduce the fire 90 hazard. These objects are accomplished by applying to the outer surface of the covering 13 a coating 16 of stearin pitch or other water-proof and fire-repellant compound such as the compound 12 above described.

If stearin pitch is used to form the outer coating 16 it will remain more or less sticky and thus make the treated conductor mean to handle, but this objection is completely overcome by applying to the sticky surface a thin

coating 17 of paraffin wax or the like to impart a slick finish to the covering as fully described and claimed in my Patent No. 1,635,829 granted July 12, 1927.

5 It will be seen from the foregoing that the coating of stearin pitch or the like applied to the rubber jacket 11 in accordance with the present invention protects that jacket from fire and from the deteriorating action of 10 the air while at the same time it serves to adhesively secure the covering 13 to the jacket 11 so that the covering will not slip back and expose the rubber. Furthermore, the presence of stearin pitch upon both the inner and 15 outer face of the protecting sheath 13 increases the waterproof and fire-repellant properties of the covered conductor.

What is claimed is:

An article of manufacture comprising, an 20 electric conductor having a protecting jacket formed of a homogeneous compound of flexible insulating material deposited about the conductor and to the outer surface of which is applied a moisture-proof and fire- 25 repellant coating of stearin pitch, a covering of fibrous material applied over said pitch coating and secured to the underlying jacket by the pitch, a second moisture-proof and fire-repellant coating of stearin pitch applied 30 to the outer surface of said fibrous covering, and a film of wax-like material applied over said second coating.

In testimony whereof, I have signed my name to this specification.

35 OTTO A. FREDERICKSON.

40

45

50

55